# EUROPEAN PATENT APPLICATION

(11) **EP 0 994 063 A1**
(43) Date of publication of application: **19.04.2000**
(21) Application number: 99830601.3
(22) Date of filing: 23.09.1999
(51) Int. Cl.: B65H 75/10

(54) **Support core for rolls of continuous sheet materials, particularly for the paper industry**

(30) Priority: 16.10.1998 IT LU980013
(71) Applicant: Sartini, Fausto, 55032 Castelnuovo Garfagnana (IT)
(72) Inventor: Sartini, Fausto, 55032 Castelnuovo Garfagnana (IT)
(74) Representative: Bardini, Marco Luigi

(57) **Abstract**

A support core for rolls of continuous sheet materials made of a plastic material comprising HD polyethylene with a flame retardant additive and fillers such as calcium carbonate, talc and carbon block.

## Description

The present invention relates to a support core for rolls of continuous sheet materials, which is especially used, though not exclusively, with advantage in the paper industry.

Paper manufacturing farms, both those which produce paper webs (tissue) and those which convert them into finished products, (such as paper for sanitary or food use) currently use cardboard cores as a support for rolling up their product. Cardboard cores have, nevertheless, several inconveniences. First, the cardboard constituting the cores is not recyclable: in fact, in order to ensure a sufficient strength to the cores, special binders are added to the pulp that cannot be removed by the usual pulping process. As a consequence, these cores are disposed as a special waste. Furthermore, due to the high unrolling speed, cardboard cores cannot be reused in no more than one or, at the most, two working cycles.

It must also be taken into account that, due to their hygroscopicity, cardboard cores are easily perishable and, due to their poor mechanical strength, tend to squash and ovalize, thus becoming unusable.

Finally the cardboard cores presently in use are easily flammable and constitute a further cause of fire in an environment, such as that of the paper industry, where this risk is already very high.

Therefore there is a strong, unsatisfied need in this field to have available an alternative to the cardboard cores presently in use to overcome the prior art drawbacks.

It is an object of the present invention to provide a support core for rolls of continuous sheet materials, such as paper, having excellent mechanical strength and dimensional stability and capable of being used a number of times much higher than that allowed by the support cores presently in use.

Another object of the present invention is to provide a support core for rolls of continuous sheet materials of the above mentioned type, which can be recycled at the end of its useful life.

A further object of the present invention is to provide a support core of the above mentioned type which is stable in the presence of humidity and fire-resistant.

The above objects are achieved with the support core for rolls of continuous sheet materials according to the present invention, the main feature of which is the fact that it is made of a plastic material comprising high-density filled polyethylene with a density comprised between 0,945 and 0,962 g/cc, as well as a flame-retardant in a weight percentage not higher than 2%. As a filler, there may be advantageously used talc (0-36%) to increase the stiffness, calcium carbonate (0-30%) to improve the workability, carbon black (0-2,5%) to improve the resistance to the atmospheric agents and UV rays, thus allowing an outdoor storage. These additives can be used alone or in combination. As a flame-retardant additive a commercially available masterbatch can be used such as those based on organic bromide compounds or nitrogen-phosphorous compounds, for instance those produced by the firm VIBA of Tradate (Varese, Italy), or equivalent flame-retardant products well-known to a person skilled in the art.

The melt index of the polyethylene is comprised between 0,05 and 0,5 (basis 5 Kg, 190°C).

The composition of the mixture of raw material used for the manufacture of the support cores according to the invention may vary as a function of the specific needs of the user, taking also into account the thickness and the requested degree of stiffness. Although the composition may vary according to the above mentioned requirements, a particularly preferred weight composition for the manufacture of support cores is the following:

| | |
|---|---|
| HDPE | 80% |
| Flame retardant additive | 1% |
| Talc | 8% |
| Calcium carbonate | 9% |
| Carbon black | 2% |

With the above mixture there can be produced support cores having, for example, a length up to 15 m, a thickness from 3 to 30 mm and a diameter from 16 to 500 mm, usable for example for producing paper rolls of a weight up to 3 tons.

The polyethylene support cores according to the present invention exhibit significant advantages over the conventional cardboard cores and in particular greater resistance, possibility of being reused for several times, easy of being disposed, resistance to humidity and chemicals. Moreover they are fireproof and have an high dimensional stability. The latter property allows the cores to be reused for several times thanks to the low risk of deformation to which they are subjected. Furthermore, it must be taken into account that the above advantages are achieved thanks to the special mixture of materials, which the cores of the invention are made of, without adversely affecting the cost of the product that can be marketed at competitive prices with respect to the conventional cardboard cores.

The support cores according to the present invention will be put on the market in a wide range of thicknesses and diameters as requested by the specific used which they are destined to. The use of the support cores of the invention is not limited to the paper industry, but can be extended to other fields such as textile industry.

Variations and/or modifications can be brought to the support core for rolls of continuous sheet materials according to the present invention, without departing from the scope of the invention itself as set forth in the appended claims.

## Claims

1. A support core for continuous sheet materials to be rolled up on it characterized in that it is made of high density polyethylene, said density being comprised between 0,945 and 0,962 g/cc and comprising a flame retardant additive and a filler material.

2. The support core according to claim 1, in which said filler material is selected from talc, calcium carbonate, carbon black, their mixtures and functionally equivalent products.

3. The support core according to claim 2, in which said high density polyethylene is a compound with the following weight percent composition:
| | |
|---|---|
| HD polyethylene | 70-98% |
| Flame retardant additive | 0,5- 2% |
| Talc | 0-36% |
| Calcium carbonate | 0-30% |
| Carbon black | 0-2,5% |
